

## UNITED STATES PATENT OFFICE

2,256,923

## METHOD FOR MAKING ALUMINUM WOOL

Charles E. Galvin, Springfield, Ohio; Reece M. Carey, administrator of said Charles E. Galvin, deceased

No Drawing. Application June 21, 1940,  
Serial No. 341,782

7 Claims. (Cl. 148—11.5)

My invention relates to the practice of making aluminum wool as a product similar in structure to steel wool except that it is made of aluminum.

It has long been known as desirable to make aluminum wool, for the reason that aluminum is not as abrasive as steel wool, and does not rust. The difficulty has been two-fold, however, so that no aluminum wool of commercial value has been produced. In the first place the making of steel wool has been to cut long shavings or filaments from a moving strand of steel wire. This will not work with aluminum wire, because the shavings break due to brittleness thereof, the softness of the wire is such that the shaving or cutting knives dig into the wire and gouge or break it.

Also such is the work hardening effect of shaving aluminum into fine shreds that the wool will break up into fragments with any handling thereof such as required to fabricate it into pads or the like.

It is known that wool can be cut from tubes of steel by the use of suitable cutters operating against the end of the tube. By using aluminum tubes and cutting the wool from the ends of the tubes which are slowly moved with reference to the cutters, I have been able to solve the problem of making the wool of aluminum initially.

I then take the wool as a mass, and place it in a furnace under conditions open to the atmosphere but not open to the products of combustion and bring it to a temperature of from 600 to 900° F. I can also gently lead a skein of the wool through a heated tube to gain the same effect continuously.

If the temperature is as low as 500° F. the effect of heating is not appreciated. If the temperature of around 1000° F. is reached by the wool, there is a deleterious effect. The time of treatment is not important provided all of the wool reaches the desired temperature. In my experience a temperature of 700° F. for a minute in a muffle furnace will produce the result.

My heat treatment will make the aluminum wool dead soft, such that it becomes less fragile than steel wool. It can be formed into pads, packed between frames to form filters, and generally fabricated as desired.

When used as an abrasive it will not scratch glass or polished chrome, or nickel surfaces. It will not leave particles in a sink after use with dishes or pans, which spots will rust and form specks which are unsightly. It will not form slivers which get into the fingers.

In filtering screens it will not corrode under moisture conditions.

It will be apparent that if someone should discover a practice feasible for making wool from aluminum wire that my practice of heat treatment before fabricating would be useful. However, I have been unable to make wool in this fashion and believe that the only practical way is to cut the wool from heavy cross sections as distinguished from attempting to gouge it out of a moving strand, lengthwise thereof.

Having thus described my invention what I claim as new and desire to secure by Letters Patent, is:

15. 1. The method of making wool from aluminum which consists of forming thin elongated cuttings from a starting body of the material, and then without working the resulting wool, raising its temperature above 500° F. sufficiently to remove the work hardening effect resulting from the cutting operation.
20. 2. The method of making wool from aluminum which consists of forming thin elongated cuttings from a starting body of the material, and then without working the resulting wool, raising its temperature above 500° F. sufficiently to remove the work hardening effect resulting from the cutting operation, the cuttings being made from a cross section of the starting body as distinguished from cuttings lengthwise of such body.
25. 3. The method of making wool from aluminum which consists of forming thin elongated cuttings from a starting body of the material, and then without working the resulting wool, raising its temperature above 500° F. sufficiently to remove the work hardening effect resulting from the cutting operation, the said temperature being below about 1000° F.
30. 4. The method of making wool from aluminum which consists of forming thin elongated cuttings from a starting body of the material, and then without working the resulting wool, raising its temperature above 500° F. sufficiently to remove the work hardening effect resulting from the cutting operation, the said heating being carried out subject to the atmosphere as distinguished from vacuum or reducing conditions.
35. 5. The method of making wool from aluminum which consists of forming thin elongated cuttings from a starting body of the material, and then without working the resulting wool, raising its temperature above 500° F. sufficiently to remove the work hardening effect resulting from the cutting operation, the cuttings being made from a cross section of the starting body as

distinguished from cuttings lengthwise of such body and the upper limit of temperature to which the wool is raised being 1000° F.

6. The method of making wool from aluminum which consists of forming thin elongated cuttings from a starting body of the material, and then without working the resulting wool, raising its temperature above 500° F. sufficiently to remove the work hardening effect resulting from the cutting operation, the cuttings being made from a cross section of the starting body as distinguished from cuttings lengthwise of such body, the said heating being carried out subject to the atmosphere as distinguished from vacuum or reducing conditions and the upper 15

limit of temperature to which the wool is raised being 1000° F.

7. The method of making wool from aluminum which consists of forming thin elongated cuttings from a starting body of the material, and then without working the resulting wool, raising its temperature above 500° F. sufficiently to remove the work hardening effect resulting from the cutting operation, the cuttings being made from a cross section of the starting body as distinguished from cuttings lengthwise of such body, the heating being to between 600 and 900° F.

CHARLES E. GALVIN.